

March 11, 1947.

W. S. NUTTER

2,417,320

WOVEN TEXTILE FABRIC

Filed Jan. 25, 1946



*Invantor:  
William S. Nutter,  
By Heard Smith & Waite  
Attorneys*

## UNITED STATES PATENT OFFICE

2,417,320

## WOVEN TEXTILE FABRIC

William S. Nutter, Sanford, Maine, assignor to  
Goodall-Sanford, Inc., Sanford, Maine, a cor-  
poration of Maine

Application January 25, 1946, Serial No. 643,465

1 Claim. (Cl. 139—427)

1

The object of this invention is to present a novel woven textile flat fabric particularly suitable for use for men's, and women's summer clothing as well as for draperies and other purposes in which animal, cotton and rayon fibers are so blended together and disposed as to be substantially indistinguishable and in which the body of the fabric is well balanced, crush resistant and of a springy character rendering it particularly adaptable for use in clothing.

The object of the invention also is to present such a fabric which should be durable, washable, and have an even uniform face.

The nature and objects of the invention will appear more fully from the following specification and be particularly pointed out in the claim.

The animal fiber employed is preferably mohair, the well-known characteristics of which render it a highly valuable factor in summer clothing, draperies and similar material, but such fiber is expensive and its advantages are available in a fabric when it forms but a part thereof. The cotton and rayon fibers also have well-known desirable characteristics in fabrics; among other things the cotton giving strength and the rayon having springy characteristics and when in the filament form giving great strength. In this invention by reason of a novel arrangement and distribution of these three fibers a fabric of highly desirable characteristics is obtained and in which the three fibers are so blended and disposed that they are substantially indistinguishable at the face of the fabric.

These results are secured and the fabric will balance by forming the fabric of regularly interwoven warp and filling yarns, each of which has substantially the same count and in which these warp and filling yarns have certain definite composition and characteristics.

The drawing illustrates a portion of a fabric embodying a preferred form of the invention. But as it is practically impossible to make an accurate drawing it will be understood that the illustration is much enlarged with the yarns separated and is only of a schematic nature to indicate the general principle involved.

The warp yarn is a two-ply yarn. One ply of this warp yarn is a single cotton yarn having relatively, with respect to the other ply, a low count and low twist. The other ply is a rayon

5  
10  
15  
20  
25  
30  
35  
40  
45

filament yarn having a relatively high count with respect to the first ply and, as in the case of all filament yarns, hardly any twist. A desirable composition of this warp yarn is to have the first ply a single cotton yarn of about 16 count, and the other ply a rayon filament yarn of about 150 denier equivalent to about 35 cotton count. The standard twist of a single 16 cotton yarn is low and the standard twist of the filament rayon yarn is very low. In the twisting of these plies together by reason of their characteristics, the rayon ply is buried in the soft cotton ply and acts to give the desired strength for the warp and also to give springiness to the entire fabric and to assist in resisting crushing.

The filling yarn is made of substantially the same count and, therefore, substantially the same size as the warp resultant yarn so as to balance and stabilize the fabric. This yarn is composed substantially of three parts animal fiber, preferably mohair, and one part of staple rayon fiber, and these fibers are spun together as a single yarn of standard twist by the process such as disclosed in the patents to Nutter, 2,016,387, October 8, 1935, and Nutter et al., 2,358,656, September 19, 1944.

The count of the warp yarn, a two-ply single 16 cotton and 150 denier rayon filament given as an illustration, is about equal to 11 on the cotton or 14 on the worsted system. The single filling yarn should balance with the warp yarn and thus be of substantially the same count, but if anything on the larger side and may be about 9½ on the cotton or 13 on the worsted system.

35. This arrangement and disposition of the three different fibers renders them in the cloth when woven practically indistinguishable. When mohair is employed, it enables practically 80% of the entire fleece including the kemp to be employed.

When the viscose rayon is employed the entire fabric may be dyed in the piece with the dye taken satisfactorily by all three fibers, and with the rapid progress being made in the development of dyes, it is expected that other types of rayon when employed in the fabric may also take the dye along with the other types of fiber.

The fabric made in accordance with this invention presents an even uniform face with the three types of fibers so disposed as to be sub-

stantially indistinguishable. The body of the fabric is springy, crush resistant and well balanced. The fabric is durable particularly adapted for wear in clothing and is unaffected by washing or laundering. At the same time it is economical and readily manufactured at low cost but is of high quality due to the presence of the substantial amount of mohair or animal fiber.

Having thus described the invention, what is claimed as new, and desired to be secured by 10 Letters Patent, is:

A woven textile flat fabric composed of animal, cotton and rayon fibers presenting an even uniform face with the several types of fibers so disposed as to be substantially indistinguishable and 15 presenting a springy crush-resistant well balanced body secured by and consisting of regularly interwoven warp and filling yarns each of substantially the same count in which the warp is a two-ply yarn one ply of which is a relatively 20 low count low twist single cotton yarn and the

other ply of which is a relatively high count rayon filament yarn well buried in the first ply and in which the filling is composed of substantially three parts animal fiber and one part staple rayon fiber spun together as a single yarn of standard twist.

WILLIAM S. NUTTER.

#### REFERENCES CITED

The following references are of record in the file of this patent:

#### UNITED STATES PATENTS

| Number    | Name         | Date          |
|-----------|--------------|---------------|
| 1,131,259 | Nutter       | Mar. 9, 1915  |
| 2,112,123 | Tenney       | Mar. 22, 1928 |
| 2,122,175 | Coulter, Jr. | June 28, 1938 |

#### FOREIGN PATENTS

| Number  | Country | Date          |
|---------|---------|---------------|
| 498,954 | British | Jan. 22, 1938 |